



US005901337A

# United States Patent [19]

[19]

Rhodes et al.

[11] Patent Number: 5,901,337

[45] Date of Patent: May 4, 1999

- [54] **METHOD FOR VACUUM LOADING**

[75] Inventors: **Terry C. Rhodes**, Pittsburgh; **Henry E. Brinzer, Jr.**, Imperial; **Frank J. Rizzo**, McMurray, all of Pa.

[73] Assignee: **Crucible Materials Corporation**, Syracuse, N.Y.

[21] Appl. No.: 09/124,236

[22] Filed: **Jul. 29, 1998**

### Related U.S. Application Data

- [62] Division of application No. 08/627,547, Apr. 4, 1996.  
[51] **Int. Cl.<sup>6</sup>** ..... **B22F 3/00**  
[52] **U.S. Cl.** ..... 419/30; 419/38  
[58] **Field of Search** ..... 419/30, 38

[56] **References Cited**

## U.S. PATENT DOCUMENTS

- |           |         |                             |
|-----------|---------|-----------------------------|
| 3,042,594 | 7/1962  | Hauth .                     |
| 3,892,030 | 7/1975  | De Pierre et al. .          |
| 4,056,368 | 11/1977 | Rozmus ..... 55/2           |
| 4,104,061 | 8/1978  | Roberts .                   |
| 4,113,240 | 9/1978  | Klein ..... 266/252         |
| 4,348,212 | 9/1982  | Rozmus ..... 55/2           |
| 4,388,088 | 6/1983  | Rozmus ..... 55/101         |
| 4,632,702 | 12/1986 | DiGiambattista ..... 75/228 |
| 4,642,218 | 2/1987  | Rice ..... 419/11           |
| 4,647,426 | 3/1987  | Fiorentino ..... 419/31     |
| 4,762,679 | 8/1988  | Gegel et al. ..... 419/28   |

- |           |         |                 |       |        |
|-----------|---------|-----------------|-------|--------|
| 4,836,978 | 6/1989  | Watanabe et al. | ..... | 419/10 |
| 4,940,404 | 7/1990  | Ammon et al.    | ..... | 419/28 |
| 4,999,157 | 3/1991  | Nishio et al.   | ..... | 419/68 |
| 5,039,476 | 8/1991  | Adachi et al.   | ..... | 419/13 |
| 5,069,868 | 12/1991 | Tokiai et al.   | ..... | 419/23 |
| 5,217,664 | 6/1993  | Feichtinger     | ..... | 264/56 |
| 5,269,830 | 12/1993 | Rabin et al.    | ..... | 75/246 |
| 5,330,704 | 7/1994  | Gilman          | ..... | 419/60 |
| 5,451,244 | 9/1995  | Castledine      | ..... | 75/243 |

## OTHER PUBLICATIONS

Flécher et al., "Vacuum Degassing of Metal Powders," Int'l. Journal of Powder Metallurgy and Powder Tech., vol. 19, No. 4, 1983, pp. 269-267.

Haeussermann et al., "Dynamic Powder Degassing—Principles and Application," Leybold—Heraeus GmbH, Germany.

*Primary Examiner*—Ngoclan Mai  
*Attorney, Agent, or Firm*—Finnegan, Henderson, Farabow,  
Garrett & Dunner, L.L.P.

[57] ABSTRACT

A method and apparatus for loading tool steel and high speed steel powder to a deformable mold for compacting is disclosed. The particles are exposed to a uniform vacuum during transfer from a sealed container through a sealed conduit and into a sealed deformable mold. By this method and apparatus, the particles are uniform throughout the container and substantially free of impurities, without requiring conventional outgassing.

## 7 Claims, 1 Drawing Sheet





## METHOD FOR VACUUM LOADING

This is a division of application Ser. No. 08/627,547, filed Apr. 4, 1996, currently allowed, the specification of which which is incorporated herein by reference.

### BACKGROUND OF THE INVENTION

#### 1. Brief Description of the Invention

The present invention relates to a method for loading tool steel and high speed steel powder into a deformable mold for compacting, with the powder during transport to the mold being under dynamic, uniform vacuum.

#### 2. Brief Description of the Prior Art

Incident to the powder-metallurgy production of tool steel and high speed steel articles, prealloyed particles of the composition from which the article is to be made are loaded into a deformable container. This deformable container is then sealed and the prealloyed particles therein are consolidated by hot isostatic pressing within a gas-pressure vessel. To achieve the desired product quality, particularly from the standpoint of uniformity of microstructure and the absence of deleterious impurities, such as oxides, it is important that the powder be free of these impurities at the time of compacting. This is typically achieved by outgassing the deformable mold after the powder has been loaded therein and before sealing for consolidation as by hot isostatic pressing. As a result of the significant size and quantity of powder within the mold, it is difficult to achieve removal of impurities during outgassing uniformly with respect to the powder from top to bottom of the mold. Typically, the powder at the top of the mold, which is near the stem through which outgassing is accomplished, is at a much lower impurity level than the powder at the bottom of the mold. Consequently, after consolidation, the impurity level and thus the properties of the consolidated article may vary along the length thereof.

### SUMMARY OF THE INVENTION

It is accordingly an object of the present invention to overcome these difficulties with respect to conventional loading of tool and high speed steel powders for consolidation and to provide a method and apparatus wherein the particles are uniform throughout the container and substantially free of impurities, without requiring conventional outgassing.

This is achieved in accordance with the method of the invention by providing a desired quantity of prealloyed particles of tool or high speed steel within a sealable container. This container acts as a source of prealloyed powder particles for transfer to the deformable mold used for consolidation by hot isostatic pressing. The container is sealed and evacuated to provide a vacuum therein. Likewise, the mold, which is of a compressible material, is sealed and evacuated to likewise provide a vacuum therein. The prealloyed particles are introduced from the container to the evacuated mold through a sealed, evacuated conduit.

The evacuation of the container and the mold may be selectively performed either sequentially or simultaneously using selective valving. The compacting of the prealloyed particles within the deformable container may be performed without outgassing the mold after evacuation thereof and loading of the particles therein.

The selective evacuation of the container and mold may be achieved by the use of a single vacuum pump. The vacuum pump is isolated from the prealloyed particles.

Preferably, a dynamic vacuum is maintained within the container, mold, and conduit during introduction of the prealloyed particles from the container to the mold. This establishes a substantially uniform vacuum level for the prealloyed particles introduced through the sealed, evacuated conduit. Hence, the prealloyed particles throughout the container have been exposed to a uniform level of vacuum during the loading operation and thus exhibit uniform cleanliness along the entire length of the mold.

10 The apparatus for use in the practice of the invention includes a sealable container having a quantity of prealloyed particles therein. Means such as a vacuum pump may be used for evacuating the container to provide the vacuum therein. A sealable, compressible mold, which likewise may be evacuated by the same pump to provide a vacuum therein is adapted for sealing. A conduit is provided for transferring the prealloyed particles from the container to the mold while exposing the particles to a uniform level of vacuum during this transfer operation. In this manner, the particles are 15 protected from contamination prior to and during compacting and exhibit uniform cleanliness. Means such as a pump may be provided for selectively evacuating the container and the mold either sequentially or simultaneously. In this regard, a single vacuum pump may be employed for evacuating the container, mold, and conduit means.

20 The vacuum pump is isolated from the prealloyed particles.

25 Valves are provided within the conduit for permitting evacuation of the container and mold via the conduit by the pump, while isolating the pump from the prealloyed particles within the conduit.

30 Vibrating of the mold is provided for during transferring of the particles to the mold for purposes of increasing the packing density of the particles within the mold.

35 Transfer of the particles may be effected by a vibrating feeder integral with the conduit.

40 A weigh scale may be provided for determining the weight of the particles transferred from the container to the mold.

45 This weigh scale is preferably associated with the prealloyed particle container.

50 A level indicator may be provided in association with the mold for determining the level of the particles within the mold.

### BRIEF DESCRIPTION OF THE DRAWING

55 The single FIGURE of the drawing is a somewhat schematic assembly of an embodiment of an apparatus for use in the practice of the invention.

### DESCRIPTION OF THE PREFERRED EMBODIMENTS

With reference to the FIGURE, there is shown an example of apparatus in accordance with the invention. A prealloyed particle storage vessel designated as 10 is provided as a source of powder particles for transmission through conduit system 12 to the compressible mold 14. A vacuum pump 16 is provided in association with the conduit system 12 and vacuum manifold 32 to evacuate the conduit system as well as the storage container 10 and mold 14.

The vacuum pump 16 is isolated from the powder particles by a cyclone filtration system and element filters 18. Selective valving 20 is employed to permit the vacuum pump to evacuate the container 10 and billet 14 sequentially by evacuating one then the other or, alternatively, simulta-

neously. Compound gauges **22** and thermistor gauges **26** monitor the pressure of the conduits and pressure dampers **28** are used to regulate the gas flow rate. The conduit system **12** is of stainless steel tubing terminating at each end with O-ring gasket fittings **30** connecting the vacuum manifold **32** portion of the conduit system **12** to the container and mold.

Stainless steel flexible hoses **34** isolate the container and mold from vibration and compressive forces caused by pressure changes to allow dynamic weighing of the prealloyed particles delivered from the container to the mold. A weigh scale **36** is provided in association with the container **10** for this purpose. This weigh scale determines the weight of the particles transferred from the container to the mold.

The flow rate of the particles being transferred through the conduit system **12** is regulated by the operation of valve **38** and amplitude feeder **40**. The amplitude feeder **40** may be a conventional vibratory feeder, such as a Syntron vibrator. The level of the powder within the mold **14** is determined by a level detector **42**. When the mold is filled to the desired level, the level detector is removed and the stem **44** is heated, crimped, or swaged to achieve a mechanical seal. The cut portion is welded to achieve a reliable seal. Since the particles travelling from the container **10** through the conduit system **12** to the container **14** are subject continuously to evacuation by the action of pump **16** through manifold **32**, each particle is exposed to substantially the same vacuum level and thus the particles are uniform from top to bottom of the container **14**.

To facilitate packing density of the particles within the container **14**, a vibrating table **46** is used in association with the mold **14** to vibrate the same during the loading of powder into the mold.

What is claimed is:

1. A method for the powder metallurgy production of tool steel and high speed steel articles from prealloyed particles thereof, said method comprising providing a quantity of

prealloyed particles within a sealable container, sealing and evacuating said container to provide a vacuum therein, sealing and evacuating a compressible mold to produce a vacuum therein, and introducing said prealloyed particles from said evacuated container to said evacuated mold through a sealed evacuated conduit, and compacting said prealloyed particles within said sealed and evacuated mold, whereby contamination of said prealloyed particles is prevented prior to and during compacting.

2. The method of claim **1**, wherein said evacuating of said container and said evacuating of said mold are selectively performed either sequentially or simultaneously using selective valving.

3. The method of claim **1**, wherein said compacting of said prealloyed particles is performed without outgassing said mold after said evacuation thereof.

4. The method of claim **1**, wherein said evacuating of said container, mold, and conduit is achieved by the use of a single vacuum pump.

5. The method of claim **4**, wherein said vacuum pump is isolated from said prealloyed particles.

6. The method of claim **1**, wherein a dynamic vacuum is maintained within said container, mold, and conduit during said introducing of said prealloyed particles from said container to said mold.

7. The method of claim **6**, wherein said dynamic vacuum maintained within said container, mold, and conduit during said introducing of said prealloyed particles from said container to said mold establishes a substantially uniform vacuum level for said prealloyed particles introduced through said sealed, evacuated conduit, whereby said prealloyed particles throughout said container have been exposed to a uniform level of vacuum and thus exhibit uniform cleanliness.

\* \* \* \* \*